

## UNITED STATES PATENT OFFICE

2,227,516

WAX PAPER SHEET AND COATING  
THEREFORRandolph Spencer Soanes, Toronto, Ontario,  
Canada, assignor to Appleford Paper Products,  
Ltd., Hamilton, Ontario, CanadaNo Drawing. Application July 11, 1938,  
Serial No. 218,637

2 Claims. (Cl. 91—68)

This invention relates to an improved heat sealable, moisture proof, opaque wax paper sheet and to an improved wax composition coating for paper sheets or the like, which coating possesses the capacity when applied to the sheet of rendering the coated sheet opaque, moisture resistant, and heat sealable according to accepted commercial methods.

Waxed or coated sheets of this character are commonly used as wrappers for food stuffs, such as bread, cake and the like. Such coatings usually consist in large part of wax such as paraffin wax.

Heretofore waxed paper sheets have been of two kinds, namely, transparent or semi or partially transparent waxed sheets and opaque waxed sheets. Paraffin wax which is commonly used as a coating material has a tendency to increase the transparency of the base sheet to which it is applied and unloaded sulphite tissue which is commonly used as a base sheet to receive the coating is more nearly transparent following the application of the coating than was the uncoated base sheet. Such sheets have a wide field of use and are marketed in large quantities. It is frequently desirable, however, to provide a wax sheet which is opaque and to provide an opaque wax paper sheet it has heretofore been the practice to employ an opacifying agent as a filler or loading agent in the fabrication of the base sheet. Titanium dioxide ( $TiO_2$ ) because of its high index of refraction and the desirable white color which it imparts to the sheet has been used as such filler. Such loaded base sheet being substantially opaque was then treated with a wax, such as paraffin wax, to form a waxed opaque sheet.

An object of my invention is to provide an opaque (preferably pure white) moisture resistant, flexible, heat sealable wax composition coated sheet of paper or the like wherein the characteristics above enumerated reside in the coating.

I have developed a composition consisting in large part of paraffin wax with other suitable ingredients hereinafter specified, which composition may be applied in the conventional manner in a hot melt coating to an unloaded sulphite sheet or other suitable base sheet to produce a coated sheet which is opaque, moisture resistant, heat sealable, and possesses a high degree of pliability. Such composition coating may be applied to one or both sides of the sheet or to localized areas thereof.

Various decorative and novelty effects may be produced in an opaque wax sheet through the use of my improved coating as compared with the

opaque wax sheet where the opacity is due to the opacity of the base sheet. My improved sheet may have localized areas of transparency or translucency as compared with its otherwise opaque areas. One surface may carry the opaque coating while the opposite surface may carry the conventional so-called transparent wax coating. The base sheet may have such opposite surface printed or decorated as desired before coating with the transparent wax coating so that the print or decoration will appear on the coated sheet.

I may use an ordinary sulphite unloaded sheet as the base sheet to receive my improved coating. Because of the absorbency of such a base sheet and the character of the coating a particularly secure bond is formed by the coating with the base sheet. If desired, however, loaded or sized paper sheets may be used. If grease resistance is desired a glassine base sheet may be used. Cellophane or the like might even be used. My coating is of such a character as to form a particularly secure bond with any suitable base sheet and its high degree of flexibility and adhesion prevents cracking, breaking, or peeling of the coating from the base sheet as the sheet is wrapped or folded in use.

In one preferred form of my invention as applied to bread wrappers the paper sheet, printed as desired, is coated on the printed side with paraffin wax or other suitable hot melt coating of reasonable transparency and on the reverse side with my improved composition. Such operation may be advantageously carried out in a waxing machine of the Meyer type which permits opposite sides of the sheet to be coated with different compositions. Through the employment of suitable mechanism it is possible to produce a sheet possessing one or more bands of greater or less transparency in the direction of motion of the sheet and in marked contrast with the opacity of the remainder of the sheet. The printing will stand out in marked contrast against the pure white background enhanced if desired by a transparent coating.

The composition which I propose to employ comprises a suitable wax such as paraffin wax carrying in suspension a suitable pigment, such as titanium dioxide.  $TiO_2$  will not remain in suspension in molten paraffin wax alone. The viscosity of molten paraffin is low as is its specific gravity.  $TiO_2$  settles down very quickly in molten paraffin alone but I have found that if certain substances of a rubbery consistency, such as natural rubber or certain synthetic materials possess-

ing similar characteristics are added in very small quantity to the molten paraffin and placed in solution or what appears to be in solution therein that the  $TiO_2$  will then remain in suspension for such period of time as to make the composition readily applicable to paper sheets as a hot melt coating.

I prefer to mix a small amount, for example, one to five parts of rubber, which may be in the form of crepe rubber sheets cut up fine, or smoked rubber sheets so disintegrated, with 100 parts of wax, which wax may be in the form of paraffin wax. The rubber may be mixed with a relatively small amount of paraffin wax and stirred or otherwise incorporated therewith until it appears to go into solution therein and then this mixture may be reduced by the addition of the remaining paraffin to make up the 100 parts.

Whether the rubber actually goes into solution or a very fine dispersion is open to question but to all appearances it goes into solution and where the word "solution" is used herein as referring to the rubber going into solution in the paraffin such interpretation is intended.

25 A suitable pigment, ( $TiO_2$  has been found highly suitable) is then added to the paraffin-rubber solution and incorporated therein by passing the mixture through a paint mill or such incorporation is obtained in some other approved 30 manner. The pigment is so thoroughly incorporated in the mixture that it will remain in suspension for several hours and for such an appreciable period of time that the coating may be used as a hot melt coating for paper with the pigment uniformly and finely distributed therethrough so that the coated sheet presents a uniform opaque appearance without spots or blotches in pigmentation.

Pigment may be added in varying amounts depending upon the degree of pigmentation desired. 40 Sheets of varying opacity are used by the paper products manufacturer and it is obvious that the amount of opacifying substance could be varied as desired. Appreciable opacity is produced with 45 the addition of three parts of the  $TiO_2$  with 100 parts of paraffin wax but to produce a substantially satisfactory commercially desirable high order of opacity of the wax sheet I have found it suitable to add fifteen parts of pigment in the 50 100 part mixture of the character above set forth. The percentage of  $TiO_2$  may of course be varied not only depending on the degree of opacity desired and the character of the base sheet used but upon whether one or both surfaces of the 55 base sheet are to be coated therewith and upon the thickness of the coating layer to be applied. It is readily possible to determine the amount required for the result sought. The resulting liquid mixture is sufficiently fluid to be readily 60 applied as a thin wax coating to a paper sheet either as a hot melt or in any other conventional manner. The pigment is so finely divided and distributed throughout the wax that the sheet presents a uniform pigmentation.

65  $TiO_2$  is available in various commercial forms classified by the manufacturers as MO:HO: and WD. I have found the form known as TITANOX-A-MO very suitable but the other forms also are suitable. Other pigments may be employed. For example, zinc oxide though having a lower index of refraction and consisting of less finely divided particles is suitable for use. If zinc oxide is used it will be desirable to increase the percentage of pigment, for example, one-third 70 over that of  $TiO_2$ .

The substance of rubbery consistency in addition to serving to maintain the pigment in suspension in the paraffin also increases the security of the hot seal and increases substantially the anchorage of the coating upon the paper and increases substantially the flexibility of the coated sheet. Only a small amount of rubber is required. As low as one part to 100 parts of paraffin has an appreciable effect. Five parts of rubber to 100 parts of paraffin has proved to be ample and two to three parts has proved satisfactory.

It has been found that certain synthetic materials of a rubbery consistency may be substituted for the rubber particles of crepe or smoked rubber sheets. These synthetic substances might not even be termed true synthetic rubber. An example of such a synthetic material which has been found suitable is the polymer of iso-butylene (2 methyl propylene) known as Vistanex-Medium. In using this synthetic substance I have found it desirable to add a small amount of sodium benzoate. The sodium benzoate when added in a small trace to the paraffin bath mixture appears to increase the period of suspension of the pigment. Sodium benzoate alone will assist in maintaining titanium dioxide in suspension in paraffin but the period of suspension attained thereby is very short as compared with the suspension period where the substance of a rubbery consistency is used. The amount of sodium benzoate might be as small as one-tenth of one part up to five parts in a mixture of approximately 100 parts.

35 The term "rubbery substance" or substance of a rubbery consistency is used herein to designate either natural rubber, synthetic rubber or substances of a rubbery consistency of the character specified herein.

40 Any suitable kind of wax may be used. Paraffin wax is commonly used and a preferred paraffin wax is one having a melting range of from 133° to 136° F. A. S. T. M. melting range. The melting range of the paraffin used might vary from 125° to 150° F. Animal or vegetable waxes might be used though the price and the fact that such waxes tend to develop a rancid odor make them less to be desired than paraffin.

45 A simplified method of incorporating the rubbery substance in the solution and one which I prefer is to gradually add small fragments of pale crepe rubber sheets to a solution of molten paraffin heated to approximately 20° C. above 50 its melt point while constantly subjecting said solution to violent agitation or stirring. Such agitation and temperature should be continued for the time required to bring the rubbery substance completely into solution, which should be 55 accomplished within twelve hours or less.

60 What I claim:

65 1. A paper sheet provided with a flexible opaque moisture resistant heat sealable surface coating characterized as applied to the sheet as a hot melt coating comprising a molten solution of paraffin wax and rubber carrying sufficient titanium dioxide in suspension to opacify the coating, the relative density of the molten paraffin wax and titanium dioxide being such that the titanium dioxide would not remain in suspension in the molten paraffin alone, the amount of rubber being sufficient to retain the titanium dioxide in suspension in the molten wax and being 70 within the range of one part of rubber to 3 to 7 parts of titanium dioxide in the solution, the 75

sum total of titanium dioxide and rubber not exceeding 20% of the paraffin wax.

2. A coating composition for a sheet of paper or the like comprising one hundred parts of molten paraffin wax carrying in colloidal solution one to three parts of a rubbery substance selected from a group consisting of rubber and the poly-

mer of iso-butylene (2 methyl propylene) and carrying in suspension five parts of titanium dioxide for each part of rubber and including sodium benzoate in an amount not exceeding the amount of rubber.

RANDOLPH SPENCER SOANES.